# EUROPEAN PATENT SPECIFICATION

(11) **EP 2 129 488 B1**
(45) Date of publication and mention of the grant of the patent: **29.06.2011**
(21) Application number: 08730687.4
(22) Date of filing: 26.02.2008
(51) Int. Cl.: B24B 7/00, B24B 55/10, B24D 11/02

(54) **ABRASIVE ARTICLE AND METHOD OF MAKING AND USING THE SAME**
SCHLEIFKÖRPER UND VERFAHREN ZU DESSEN HERSTELLUNG UND VERWENDUNG
ARTICLE ABRASIF ET PROCÉDÉ DE FABRICATION ET D'UTILISATION DE CELUI-CI

(30) Priority: 20.03.2007 US 688497
(43) Date of publication of application: 09.12.2009
(73) Proprietor: 3M Innovative Properties Company, Saint Paul, MN 55133-3427 (US)
(72) Inventor: WOO, Edward J.,, Saint Paul, Minnesota 55133-3427 (US); RAMBOSEK, Thomas W.,, Saint Paul, Minnesota 55133-3427 (US); ANGADJIVAND, Seyed A.,, Saint Paul, Minnesota 55133-3427 (US); DONOVAN, Mary B.,, Saint Paul, Minnesota 55133-3427 (US); SANDERS, Rufus C. Jr.,, Saint Paul, Minnesota 55133-3427 (US); CHOU, Yeun-jong,, Saint Paul, Minnesota 55133-3427 (US)
(74) Representative: Voortmans, Gilbert J.L.
(86) International application number: PCT/US2008/054931
(87) International publication number: WO 2008/115663

(56) References cited:
- US-A1- 2001 023 168
- US-A1- 2007 066 197

## Description

### BACKGROUND

Abrasive articles are used in industry for abrading, grinding, and polishing applications. They may be obtained in a variety of converted forms, such as belts, discs, sheets, and the like, in many different sizes.

Generally, when using abrasives articles in the form of "sheet goods" (i.e., discs and sheets), a back-up pad is used to mount or attach the abrasive article to the abrading tool. One type of back-up pad has dust collection holes connected by a series of grooves. The dust collection holes are typically connected to a vacuum source to help control particles such as, for example, swarf (as used herein, the term "swarf" refers loose material such as dust and debris generated during abrading processes) build-up on the abrading surface of the abrasive article. Removing swarf from the abrading surface is known to improve the performance of the abrasive article.

Some abrasive tools have integral vacuum systems with dust collection means. The extracting and holding capabilities of these abrasive tools have been limited, in part, due to the suction requirements of current abrasive disks that their related back-up pads require.

In some abrasive tool configurations, dust is collected in a complex collection system through a hose connected to the abrasive tools. Dust collection systems, however, are not always available for the abrasive tool operator. Further, the use of dust collection systems requiring hoses may be cumbersome and may interfere with the operator's manipulation of the abrasive tool.

The document US-A-2001/023168 discloses the nearest prior art. In particular, the document discloses an abrasive article and a method for its production, said abrasive article comprising: a porous abrasive member comprising: an abrasive layer proximate and affixed to a first surface of a substrate, the abrasive layer comprising a plurality of abrasive particles affixed to the first surface of the substrate by at least one binder, wherein the abrasive layer has an outer abrasive surface, wherein the substrate has a second surface opposite the first surface of the substrate, and wherein a plurality of openings extend from the outer abrasive surface to the second surface of the substrate.

### SUMMARY

In one aspect, the present invention provides an abrasive article comprising:
a porous abrasive member comprising: an abrasive layer proximate and affixed to a first surface of a substrate, the abrasive layer comprising a plurality of abrasive particles affixed to the first surface of the substrate by at least one binder, wherein the abrasive layer has an outer abrasive surface, wherein the substrate has a second surface opposite the first surface of the substrate, and wherein a plurality of openings extend from the outer abrasive surface to the second surface of the substrate;
a first nonwoven filter medium having a first surface and a second surface opposite the first surface, wherein the first surface of the first nonwoven filter medium is proximate and affixed to the second surface of the substrate, wherein the first nonwoven filter medium comprises a plurality of fibers; and
a second nonwoven filter medium having a first surface and a second surface opposite the first surface, wherein the first surface of the second nonwoven filter medium is proximate and affixed to the second surface of the first nonwoven filter medium, and wherein the second nonwoven filter medium comprises a plurality of fibers;
wherein the plurality of openings cooperate with the first nonwoven filter medium to allow the flow of particles from the outer abrasive surface to the second nonwoven filter medium, and wherein, in an unused state, the at least a portion of the abrasive article exhibits a pressure drop according to the Pressure Drop Measurement Test in a range of from 0.2 to 20 millimeters of water.

In another aspect, the present invention provides a method of making an abrasive article, the method comprising:
providing a porous abrasive member comprising: an abrasive layer proximate and affixed to a first surface of a substrate, the abrasive layer comprising a plurality of abrasive particles affixed to the first surface of the substrate by at least one binder, wherein the abrasive layer has an outer abrasive surface, wherein the substrate has a second surface opposite the first surface of the substrate, and wherein a plurality of openings extend from the outer abrasive surface to the second surface of the substrate;
providing a first nonwoven filter medium, the first nonwoven filter medium having a first surface and a second surface opposite the first surface, wherein the first nonwoven filter medium comprises a plurality of fibers, and wherein the first surface of the first nonwoven filter medium is proximate the second surface of the substrate;
providing a second nonwoven filter medium, the second nonwoven filter medium having a first surface and a second surface opposite the first surface, wherein the second nonwoven filter medium comprises a plurality of fibers, and wherein the first surface of the second nonwoven filter medium is proximate the second surface of the first nonwoven filter medium;
affixing the first nonwoven filter medium to the second surface of the substrate; and
affixing the second nonwoven filter medium to the first nonwoven filter medium;
wherein the plurality of openings cooperate with the first nonwoven filter medium to allow the flow of particles from the outer abrasive surface to the second nonwoven filter medium, and wherein, in an unused state, at least a portion of the abrasive article exhibits a pressure drop according to the Pressure Drop Measurement Test in a range of from 0.2 to 20 millimeters of water.

In yet another aspect, the present invention provides an abrasive article comprising:
a porous abrasive member comprising: an abrasive layer proximate and affixed to a first surface of a substrate, the abrasive layer comprising a plurality of abrasive particles affixed to the first surface of the substrate by at least one binder, wherein the abrasive layer has an outer abrasive surface, wherein the substrate has a second surface opposite the first surface of the substrate, and wherein a plurality of openings extend from the outer abrasive surface to the second surface of the substrate;
a first nonwoven filter medium having a first surface and a second surface opposite the first surface, wherein the first surface of the first nonwoven filter medium is proximate and affixed to the second surface of the substrate, wherein the first nonwoven filter medium comprises a plurality of fibers, and wherein the first nonwoven filter medium has a thickness of from 1 to 25 millimeters and a bulk density of from 0.04 to 0.5 grams per cubic centimeter; and
a second nonwoven filter medium having a first surface and a second surface opposite the first surface, wherein the first surface of the second nonwoven filter medium is proximate and affixed to the second surface of the first nonwoven filter medium, wherein the second nonwoven filter medium comprises a plurality of fibers, and wherein the second nonwoven filter medium has a thickness of from 0.5 to 15 millimeters and a bulk density of from 0.04 to 0.5 grams per cubic centimeter; and
wherein the plurality of openings cooperate with the first nonwoven filter medium to allow the flow of particles from the outer abrasive surface to the second nonwoven filter medium.

In yet another aspect the present invention provides a method of making an abrasive article, the method comprising:
providing a porous abrasive member comprising: an abrasive layer proximate and affixed to a first surface of a substrate, the abrasive layer comprising a plurality of abrasive particles affixed to the first surface of the substrate by at least one binder, wherein the abrasive layer has an outer abrasive surface, wherein the substrate has a second surface opposite the first surface of the substrate, and wherein a plurality of openings extend from the outer abrasive surface to the second surface of the substrate;
providing a first nonwoven filter medium having a first surface and a second surface opposite the first surface, wherein the first surface of the first nonwoven filter medium is proximate the second surface of the substrate, wherein the first nonwoven filter medium comprises a plurality of fibers, and wherein the second nonwoven filter medium has a thickness of from 0.5 to 15 millimeters and a bulk density of from 0.04 to 0.5 grams per cubic centimeter;
providing a second nonwoven filter medium having a first surface and a second surface opposite the first surface, wherein the first surface of the second nonwoven filter medium is proximate the second surface of the first nonwoven filter medium, wherein the second nonwoven filter medium comprises a plurality of fibers, wherein the second nonwoven filter medium has a thickness of from 0.5 to 15 millimeters and a bulk density of from 0.04 to 0.5 grams per cubic centimeter;
affixing the first nonwoven filter medium to the second surface of the substrate; and
affixing the second nonwoven filter medium to the first nonwoven filter medium,
wherein the plurality of openings cooperate with the first nonwoven filter medium to allow the flow of particles from the outer abrasive surface to the second nonwoven filter medium.

In certain embodiments, the porous abrasive member comprises an apertured coated abrasive. In certain embodiments, the porous abrasive member comprises a screen abrasive. In certain embodiments, the first nonwoven filter medium and the second nonwoven filter medium are affixed to one another by needletacking or a stitch bond. In certain embodiments, the porous abrasive member is affixed to the first nonwoven filter medium by an adhesive. In certain embodiments, the first nonwoven filter medium is affixed to the second nonwoven filter medium by an adhesive. In certain embodiments, at least one of the first nonwoven filter medium or the second nonwoven filter medium comprise synthetic fibers selected from the group consisting of polypropylene fibers, polyester fibers, nylon fibers, and mixtures thereof. In certain embodiments, the substrate is selected from the group consisting of metal foil, paper, fabric, and plastic film. In certain embodiments, at least one of the first nonwoven filter medium or the second nonwoven filter medium comprises a blown microfiber web. In certain embodiments, at least one of the first nonwoven filter medium or the second nonwoven filter medium comprises an electret charge. In certain embodiments, the second surface of the substrate and the first surface of the first nonwoven filter medium are coextensive, and the second surface of the first nonwoven filter medium and the first surface of the second nonwoven filter medium are coextensive. In certain embodiments, at least one of the first or second nonwoven filter medium has a peripheral edge that is sealed along a major portion thereof. In certain embodiments, the abrasive article comprises an abrasive disc.

In certain embodiments, a porous attachment layer is affixed to the second surface of the second nonwoven filter medium. In certain embodiments, the porous attachment layer comprises a loop portion or a hook portion of a two-part mechanical engagement system. In certain embodiments, the first nonwoven filter medium, the second nonwoven filter medium, and the porous attachment layer are affixed to one another by needletacking or a stitch bond.

Abrasive articles according to the present invention are useful, for example, for abrading a surface of a workpiece by a method comprising contacting the surface with the abrasive article, and relatively moving the abrasive article and the surface to mechanically modify the surface.

Advantageously, abrasive articles according to the present invention are particularly suitable for use in those abrading applications generating appreciable amounts of particles (e.g., swarf), and in at least some embodiments, may effectively trap at least 40, 50 (i.e., a majority), 60, 70, 80, or even more than 90 percent of particles generated in such abrading applications, for example, if used in combination with a tool having a vacuum source.

As used herein,
the term "air resistance" refers to resistance of air passing through the thickness dimension of a nonwoven web or abrasive article, and, when used for comparison purposes, all air resistance values are to be measured under like conditions;
the term "nonwoven filter medium" refers to a material, having internal void space and formed substantially of a plurality of entangled and/or bonded fibers, produced by a process other than weaving or knitting; and
the term "thickness" as applied to a nonwoven filter medium refers to the thickness of the nonwoven web as measured according to ASTM D5736-95 (Reapproved 2001) "Standard Test Method for Thickness of Highloft Nonwoven Fabrics" using a pressure plate force of 0.002 pound per square inch (13.8 Pa).

### BRIEF DESCRIPTION OF THE DRAWING

Fig. 1A is a perspective view of an exemplary abrasive article according to one embodiment of the present invention, partially cut away to reveal the layers forming the article;
Fig. 1B is a schematic cross-sectional view of the abrasive article shown in Fig. 1A;
Fig. 2A is a top view of an exemplary porous abrasive member useful in abrasive articles according to the present invention;
Fig. 2B is a cross-sectional view of the porous abrasive member shown in Fig. 2A;
Fig. 3 is a top view of an exemplary porous abrasive member useful in abrasive articles according to the present invention, partially cut away to reveal the components forming the abrasive layer; and
Fig. 4 is a scale top view showing an exemplary perforation pattern 400 for a 5-inch diameter coated abrasive disc.

These figures, which are idealized, are intended to be merely illustrative of the abrasive article of the present invention and non-limiting.

### DETAILED DESCRIPTION

Fig. 1A shows a perspective view of an exemplary abrasive article 102 (shown as an abrasive disc) with a partial cutaway. As shown in Fig. 1A, the abrasive article 102 has a porous abrasive member 104, a first nonwoven filter medium 120, a second nonwoven filter medium 140, and an optional porous attachment layer 146. The porous abrasive member 104 comprises a plurality of openings that allow the flow of particles (e.g., swarf generated during an abrading process) through the porous abrasive member 104. Particles are then captured by the filter medium within the abrasive article. Optional seal 105 seals the peripheral edge 106 (shown in Fig. 1B) of first and second nonwoven filter medium 120, 140, respectively, thereby preventing lateral escape of particles not retained by the abrasive article 102.

Fig. 1B shows a schematic cross-sectional view of the abrasive article 102 shown in Fig. 1A. As shown in Fig. 1B, the abrasive article 102 comprises multiple layers. The first nonwoven filter medium 120 comprises a first surface 122 and a second surface 124 opposite the first surface 122. The second nonwoven filter medium 140 comprises a first surface 142 and a second surface 144 opposite the first surface 142. The first surface 122 of the first nonwoven filter medium 120 is proximate the porous abrasive member 104. The second surface 124 of the first nonwoven filter medium 120 is proximate the first surface 142 of the second nonwoven filter medium 140. A porous attachment layer 146 is proximate the second surface 144 of the second nonwoven filter medium 140.

The porous abrasive member and various filter medium layers of the abrasive article are affixed to one another in a manner that does not prevent the flow of particles from one layer to the next, although some partial or minor obstruction(s) to particle flow may be present. In some embodiments, the porous abrasive member and various filter medium layers of the abrasive article are affixed to one another in a manner that does not substantially inhibit the flow of particles from one layer to the next. In some embodiments, the level of particle flow through the abrasive article may be restricted, at least in part, by the introduction of an adhesive between the porous abrasive member and the first nonwoven filter medium, or the first nonwoven filter medium and the second nonwoven filter medium. The level of restriction may be minimized by applying the adhesive between layers in a discontinuous fashion such as for example, as discrete adhesive areas (e.g., atomized spray or starved extrusion die) or distinct adhesive lines (e.g., hot melt swirl-spray or patterned roll coater).

Fig. 2A shows a top view of an exemplary coated abrasive material used to form the porous abrasive member. Fig. 2B shows a cross-sectional view of a section of the porous abrasive member shown in Fig. 2A. As shown in Fig. 2B, the porous abrasive member 204 comprises a substrate 206 having a first surface 208 and a second surface 210, a make coat 214, a plurality of abrasive particles 212, and a size coat 215. As shown in Fig. 2A, the porous abrasive member 204 comprises a plurality of apertures 216 (not shown in Fig. 2B).

Fig. 3 shows a top view of an exemplary screen abrasive material used to form the porous abrasive member. Fig. 3 includes a partial cutaway to reveal the components forming the abrasive layer. As shown in Fig. 3, the porous abrasive member 304 comprises an open mesh substrate 306, a make coat 314, a plurality of abrasive particles 312, and a size coat 315. The porous abrasive member 304 comprises a plurality of openings 316 that extend through the porous abrasive member. The openings 316 are formed by openings 318 in the open mesh substrate 306.

The open mesh substrate may be made from any porous material including, for example, perforated films, nonwovens, or woven or knitted fabrics. In the embodiment shown in Fig. 3, the open mesh substrate 306 is a perforated film. The film for the substrate may be made from metal, paper, or plastic, including molded thermoplastic materials and molded thermoset materials. In some embodiments, the open mesh substrate comprises perforated or slit and stretched sheet materials. In some embodiments, the open mesh substrate comprises fiberglass, nylon, polyester, polypropylene, or aluminum.

The openings 318 in the open mesh substrate 306 may be generally square shaped as shown in Fig. 3. In other embodiments, the shape of the openings may be other geometric shapes including, for example, a rectangular shape, a circular shape, an oval shape, a triangular shape, a parallelogram shape, a polygon shape, or a combination of these shapes. The openings 318 in the open mesh substrate 306 may be uniformly sized and positioned as shown in Fig. 3. In other embodiments, the openings may be placed non-uniformly by, for example, using a random opening placement pattern, varying the size or shape of the openings, or any combination of random placement, random shapes, and random sizes.

In another aspect, a screen abrasive with a woven or knitted substrate may be used to form the porous abrasive member. A woven substrate typically comprises a plurality of generally parallel warp elements that extend in a first direction and a plurality of generally parallel weft elements that extend in a second direction. The weft elements and warp elements of the open mesh substrate intersect to form a plurality of openings. The second direction may be perpendicular to the first direction to form square shaped openings in the woven open mesh substrate. In some embodiments, the first and second directions intersect to form a diamond pattern. The shape of the openings may be other geometric shapes including, for example, a rectangular shape, a circular shape, an oval shape, a triangular shape, a parallelogram shape, a polygon shape, or a combination of these shapes. In some embodiments, the warp and weft elements are yarns that are woven together in a one-over-one weave.

The warp and weft elements may be combined in any manner known to those in the art including, for example, weaving, stitch-bonding, or adhesive bonding. The warp and weft elements may be fibers, filaments, threads, yarns or a combination thereof. The warp and weft elements may be made from a variety of materials known to those skilled in the art including, for example, synthetic fibers, natural fibers, glass fibers, and metal. In some embodiments, the warp and weft elements comprise monofilaments of thermoplastic material or metal wire. In some embodiments, the woven open mesh substrate comprises nylon, polyester, or polypropylene.

The porous abrasive member, whether a screen abrasive, a perforated coated abrasive, or otherwise, may comprise openings having different open areas. The "open area" of an opening in the porous abrasive member refers to the area of the opening as measured over the thickness of the porous abrasive member (i.e., the area bounded by the perimeter of material forming the opening through which a three-dimensional object could pass). Useful porous abrasive members typically have an average open area of at least about 0.5 square millimeters per opening. In some embodiments, the porous abrasive member has an average open area of at least about one square millimeter per opening. In yet further embodiments, the porous abrasive member has an average open area of at least about 1.5 square millimeters per opening.

The porous abrasive member, whether woven, perforated or otherwise, comprises a total open area that affects the amount of air that may pass through the porous abrasive member as well as the effective area and performance of the abrasive layer. The "total open area" of the porous abrasive member refers to the cumulative open areas of the openings as measured over the area formed by the perimeter of the porous abrasive member. Porous abrasive members have a total open area of at least about 0.01 square centimeters per square centimeter of the abrasive layer (i.e., 1 percent open area). In some embodiments, the porous abrasive member has a total open area of at least about 0.03 square centimeters per square centimeter of the abrasive layer (i.e., 3 percent open area). In yet further embodiments, the porous abrasive member has a total open area of at least about 0.05 square centimeters per square centimeter of the abrasive layer (i.e., 5 percent open area).

Typically, the porous abrasive member has a total open area that is less than about 0.95 square centimeters per square centimeter of the abrasive layer (i.e., 95 percent open area). In some embodiments, the porous abrasive member has a total open area that is less than about 0.9 square centimeters per square centimeter of the abrasive layer (i.e., 90 percent open area). In yet further embodiments, the porous abrasive member has a total open area that is less than about 0.80 square centimeters per square centimeter of the abrasive layer (i.e., 80 percent open area).

As discussed above, the porous abrasive member, whether a perforated coated abrasive, a coated screen abrasive, a nonwoven abrasive, or otherwise, comprises a plurality of abrasive particles and at least one binder. In some embodiments, the abrasive layer comprises a make coat, a size coat, a supersize coat, or a combination thereof. In some embodiments, the abrasive layer is provided, at least in part, by curing a slurry coat comprising abrasive particles in a binder precursor. Typically, a make layer of a coated abrasive is prepared by coating at least a portion of a substrate (e.g., a treated or untreated backing, open mesh, or nonwoven fiber web) with a make layer precursor comprising a first binder precursor.

The substrate may have one or more treatments (e.g., a backsize, presize, saturant, or subsize) thereon. Suitable substrates are widely known in the abrasive arts and may consist of, for example, metal foil, paper, fabric (e.g., knits, nonwovens, or wovens (including open scrims and tightly woven fabrics), woven mesh (e.g., scrim), plastic film (e.g., including thermoplastic materials such as polyester, polyethylene, and polypropylene), and combinations thereof. In some embodiments, the substrate does not have a laminate structure.

The substrate is preferably relatively thin and flexible. For example, in some embodiments, the substrate may have a thickness of less than 1 millimeter, less than 0.5 millimeter, or even less than 0.1 millimeter. In some embodiments, the perforations, holes, or other porous features extending through the thickness of the substrate have a substantially uniform cross-section throughout their length.

Abrasive particles are then at least partially embedded (e.g., by electrostatic or drop coating) to the make layer precursor comprising a first binder precursor, and the make layer precursor is at least partially cured. Electrostatic coating of the abrasive particles typically provides erectly oriented abrasive particles. In the context of the abrasive articles, the term "erectly oriented" refers to a characteristic in which the longer dimensions of a majority of the abrasive particles are oriented substantially perpendicular (i.e., between 60 and 120 degrees) to the substrate. Other techniques for erectly orienting abrasive particles may also be used.

Next, the size layer is prepared by coating at least a portion of the make layer and abrasive particles with a size layer precursor comprising a second binder precursor (which may be the same as, or different from, the first binder precursor), and at least partially curing the size layer precursor. In some coated abrasive articles, a supersize is applied to at least a portion of the size layer. If present, the supersize layer typically includes grinding aids and/or anti-loading materials.

Typically, a binder is formed by curing (e.g., by thermal means, or by using electromagnetic or particulate radiation) a binder precursor. Useful binder precursors suitable for use in make, size, supersize, and slurry coats are well known in the abrasive art and include, for example, free-radically polymerizable monomer and/or oligomer, epoxy resins, acrylic resins, urethane resins, phenolic resins, urea-formaldehyde resins, melamine-formaldehyde resins, aminoplast resins, cyanate resins, or combinations thereof. Useful binder precursors include thermally curable resins and radiation curable resins, which may be cured, for example, thermally and/or by exposure to radiation.

As is well known in the art, catalysts, initiators, and/or curatives may be used in combination with binder precursors, typically in an effective amount.

Suitable abrasive particles for the coated abrasives include, for example, any known abrasive particles or materials commonly used in abrasive articles. Examples of useful abrasive particles for coated abrasives include, for example, fused aluminum oxide, heat treated aluminum oxide, white fused aluminum oxide, black silicon carbide, green silicon carbide, titanium diboride, boron carbide, tungsten carbide, titanium carbide, diamond, cubic boron nitride, garnet, fused alumina zirconia, sol gel abrasive particles, silica, iron oxide, chromia, ceria, zirconia, titania, silicates, metal carbonates (such as calcium carbonate (e.g., chalk, calcite, marl, travertine, marble and limestone), calcium magnesium carbonate, sodium carbonate, magnesium carbonate), silica (e.g., quartz, glass beads, glass bubbles and glass fibers) silicates (e.g., talc, clays, (montmorillonite) feldspar, mica, calcium silicate, calcium metasilicate, sodium aluminosilicate, sodium silicate) metal sulfates (e.g., calcium sulfate, barium sulfate, sodium sulfate, aluminum sodium sulfate, aluminum sulfate), gypsum, aluminum trihydrate, graphite, metal oxides (e.g., tin oxide, calcium oxide), aluminum oxide, titanium dioxide and metal sulfites (e.g., calcium sulfite), metal particles (e.g., tin, lead, copper), plastic abrasive particles formed from a thermoplastic material (e.g., polycarbonate, polyetherimide, polyester, polyethylene, polysulfone, polystyrene, acrylonitrile-butadiene-styrene block copolymer, polypropylene, acetal polymers, polyvinyl chloride, polyurethanes, nylon), plastic abrasive particles formed from crosslinked polymers (e.g., phenolic resins, aminoplast resins, urethane resins, epoxy resins, melamine-formaldehyde, acrylate resins, acrylated isocyanurate resins, urea-formaldehyde resins, isocyanurate resins, acrylated urethane resins, acrylated epoxy resins), and combinations thereof. The abrasive particles may also be agglomerates or composites that include additional components, such as, for example, a binder. Criteria used in selecting abrasive particles used for a particular abrading application typically include: abrading life, rate of cut, substrate surface finish, grinding efficiency, and product cost.

Coated abrasive members may further comprise optional additives such as abrasive particle surface modification additives, coupling agents, plasticizers, fillers, expanding agents, fibers, antistatic agents, initiators, suspending agents, photosensitizers, lubricants, wetting agents, surfactants, pigments, dyes, UV stabilizers, and suspending agents. The amounts of these materials are selected to provide the properties desired. Additives may also be incorporated into the binder, applied as a separate coating, held within the pores of the agglomerate, or combinations of the above.

If not inherently porous (e.g., due to the nature of the substrate), the abrasive member may be perforated, for example, by mechanical perforation (e.g., die punching), laser perforation, any other suitable technique. Any pattern of perforations may be used. Perforations may be, for example, round or oblong, straight, arcuate, or some complex shape. There should be sufficient porosity of the porous abrasive member to allow particles (e.g., swarf) to flow from the outer abrasive surface to the first and second filter medium at a rate comparable to that at which they are generated.

Examples of commercially available apertured coated abrasive articles suitable for use as a porous abrasive member include material available under the trade designation "NORTON MULTI-AIR", from Saint-Gobain Abrasives GmbH, Wesseling, Germany, and coated abrasive discs available under the trade designation "CLEAN SANDING DISC" from 3M Company, Saint Paul. Minnesota.

In some embodiments, the first and/or second nonwoven filter media have an average thickness in a range of at least 0.5, 1, or even at least 5 millimeters up to 10 or 15 millimeters. In other embodiments, the first nonwoven filter medium may have a thickness of up to 20, or even 30 millimeters, or more. In some embodiments, the first nonwoven filter medium has an average thickness that is less than about 20 millimeters.

In some embodiments, the first and/or second nonwoven filter media have a bulk density of from 0.04 to 0.5 grams per cubic centimeter (g/cm³). For example, the first filter medium may have a bulk density of from 0.75 to 0.4 g/cm³, or from 1 to 0.3 g/cm³_{.}

In some embodiments, the first filter medium is thicker and optionally less dense than the second filter medium. In other embodiments, the second filter medium is thicker and optionally less dense than the first filter medium.

The first and/or second filter medium of the abrasive article may be electrostatically charged. Electrostatic charging enhances the filter media's ability to remove particulate matter from a fluid stream by increasing the attraction between particles and the surface of the filter medium. Non-impinging particles passing close to fibers of the filter media are more readily pulled from the fluid stream, and impinging particles are adhered more strongly. Passive electrostatic charging is provided by an electret, which is a dielectric material that exhibits a semi-permanent or permanent electrical charge. Electret chargeable polymeric materials include nonpolar polymers such as polytetrafluoroethylene (PTFE) and polypropylene.

Several methods are used to charge dielectric materials, any of which may be used to charge the filtration medium of the abrasive article, including corona discharge, heating and cooling the material in the presence of a charged field, contact electrification, spraying the web with charged particles, and impinging a surface with water jets or water droplet streams. In addition, the chargeability of the surface may be enhanced by the use of blended materials. Examples of charging methods are disclosed in U.S. Pat. Nos. RE 30,782 (van Turnhout et al.); RE 31,285 (van Turnhout et al.); 5,496,507 (Angadjivand et al.); 5,47.1,481 (Jones et al.); 4,215,682 (Kubik et al.); 5,057,710 (Nishiura et al.); and 4,592,815 (Nakao); 5,976,208 (Rousseau et al.).

Each of the first and/or second nonwoven filter media comprise a plurality of fibers.

In some embodiments, the first and/or second nonwoven filter media comprise materials having a fiber size that is less than about 100 microns in diameter, and sometimes less than about 50 microns, and sometimes less than about 1 micron in diameter.

The first and/or second nonwoven filter media may be made from a wide variety of organic polymeric materials, including mixtures and blends. Suitable filter medium includes a wide range of materials commercially available. They include polyolefins, such as polypropylene, linear low density polyethylene, poly-1-butene, poly(4-methyl-1-pentene), polytetrafluoroethylene, polychlorotrifluoroethylene; or polyvinyl chloride; aromatic polyarenes, such as polystyrene; polycarbonates; polyesters; and combinations thereof (including blends or copolymers). In some embodiments, materials include polyolefins free of branched alkyl radicals and copolymers thereof. In yet further embodiments, materials include thermoplastic fiber formers (e.g., polyolefins such as polyethylene, polypropylene, copolymers thereof, etc.). Other suitable materials include: thermoplastic polymers such as polylactic acid (PLA); non-thermoplastic fibers such as cellulose, rayon, acrylic, and modified acrylic (halogen modified acrylic); polyamide or polyimide fibers such as those available under the trade designations "NOMEX" and "KEVLAR" from E.I. du Pont de Nemours & Co., Wilmington, Delaware; and fiber blends of different polymers.

The nonwoven filter media may be formed in a web by conventional nonwoven techniques including, for example, melt blown, spunbond, carding, air laying (dry laying), or wet laying techniques. Details concerning blown microfiber webs and methods for their manufacture are well known in the art and may be found, for example, in U.S. Pat. Nos. 6,139,308 (Berrigan et al.) and 5,496,507 (Angadjivand et al.). Exemplary melt blown nonwoven filter media include bimodal blown microfiber media, for example, as described in U.S. Pat. Appln. No. 11/461136 to Brandner et al., filed July 31, 2006.

If desired, the nonwoven filter medium may have a gradient density, for example, as prepared by contacting a thermoformable nonwoven web with a hot can.

If desired, the fibers or webs may be charged by known methods, including, for example, by use of corona discharge electrodes or high-intensity electric fields. The fibers may be charged during fiber formation, prior to or while forming the fibers into the filter web or subsequent to forming the filter web. The fibers forming the second filter medium may even be charged subsequent to being joined to the first nonwoven filter medium. The second nonwoven filter medium may comprise fibers coated with a polymer binder or adhesive, including pressure sensitive adhesives.

The porous attachment layer allows air to pass through. The porous attachment layer may comprise a layer of adhesive, a fabric, a sheet material, a molded body, or a combination thereof. The sheet material may comprise, for example, a loop portion or a hook portion of a two-part mechanical engagement system. The porous attachment layer may comprise a layer of pressure sensitive adhesive with an optional release liner to protect it during handling.

In some embodiments, the porous attachment layer comprises a nonwoven, woven, or knitted loop material. The loop material may be used to affix the abrasive article to a back-up pad having a complementary mating component.

Suitable materials for a loop porous attachment layer include both woven and nonwoven materials. Woven and knit porous attachment layer materials may have loop-forming filaments or yarns included in their fabric structure to form upstanding loops for engaging hooks. Nonwoven loop attachment interface materials may have loops formed by the interlocking fibers. In some nonwoven loop attachment interface materials, the loops are formed by stitching a yarn through the nonwoven web to form upstanding loops.

Useful nonwovens suitable for use as a loop porous attachment layer include, for example, airlaids, spunbonds, spunlaces, bonded melt blown webs, and bonded carded webs. The nonwoven materials may be bonded in a variety of ways known to those skilled in the art including, for example, needle-punching, stitchbonding, hydroentangling, chemical bonding, thermal bonding, and combinations thereof. The woven or nonwoven materials used may be made from natural fibers (e.g., wood or cotton fibers), synthetic fibers (e.g., polyester or polypropylene fibers) or combinations of natural and synthetic fibers. In some embodiments, the porous attachment layer comprises nylon, polyester or polypropylene.

In some embodiments, a loop porous attachment layer having an open structure that does not significantly interfere with the flow of air through it is selected. In some embodiments, the porous attachment layer material is selected, at least in part, based on the porosity of the material.

In some embodiments, the porous attachment layer comprises a hook material. The material used to form the hook material useful in the abrasive article may be made in one of many different ways known to those skilled in the art. Several suitable processes for making hook material useful in making porous attachment layers include, for example, methods described in U.S. Pat. Nos. 5,058,247 (Thomas et al.); 4,894,060 (Nestegard); 5,679,302 (Miller et al.); and 6,579,161 (Chesley et al.).

The hook material may be a porous material such as, for example the polymer netting material reported in U.S. Pat. Appln. Publ. No. 2004/0170801 (Seth et al.). In other embodiments, the hook material may be apertured to allow air to pass through. Apertures may be formed in the hook material using any methods known to those skilled in the art. For example, the apertures may be cut from a sheet of hook material using, for example, a die, laser, or other perforating instruments known to those skilled in the art. In other embodiments, the hook material may be formed with apertures.

The porous attachment layer of the abrasive article is affixed to the filter medium in a manner that does not prevent the flow of air from the filter medium. In some embodiments, the porous attachment layer of the abrasive article is affixed to the filter medium in a manner that does not substantially inhibit the flow of air from the filter medium. The level of air flow through the porous attachment layer may be restricted, at least in part, by the introduction of an adhesive between a porous attachment layer comprising a sheet material and the filter medium. The level of restriction may be minimized by applying the adhesive between the sheet material of the porous attachment layer and the filter medium in a discontinuous fashion such as, for example, discrete adhesive areas (e.g., atomized spray or starved extrusion die) or distinct adhesive lines (e.g., hot melt swirl-spray or patterned roll coater).

Exemplary useful adhesives include both pressure sensitive and non-pressure sensitive adhesives. Pressure sensitive adhesives are normally tacky at room temperature and may be adhered to a surface by application of, at most, light finger pressure, while non-pressure sensitive adhesives include solvent, heat, or radiation activated adhesive systems. Examples of useful adhesives include those based on general compositions of polyacrylate; polyvinyl ether; diene-containing rubbers such as natural rubber, polyisoprene, and polyisobutylene; polychloroprene; butyl rubber; butadiene-acrylonitrile polymers; thermoplastic elastomers; block copolymers such as styrene-isoprene and styrene-isoprene-styrene block copolymers, ethylene-propylene-diene polymers, and styrene-butadiene polymers; poly(alpha olefins); amorphous polyolefins; silicone; ethylene-containing copolymers such as poly(ethylene-co-vinyl acetate), poly(ethylene-co-ethyl acrylate), and poly(ethylene-co-ethyl methacrylate); polyurethanes; polyamides; polyesters; epoxies; poly(vinylpyrrolidone) and vinylpyrrolidone copolymers; and mixtures of the above. Additionally, the adhesives may contain additives such as tackifiers, plasticizers, fillers, antioxidants, stabilizers, pigments, diffusing particles, curatives, and solvents.

The various layers in the abrasive article may be held together using any suitable form of attachment such as, for example, glue, pressure sensitive adhesive, hot-melt adhesive, spray adhesive, thermal bonding, needletacking, stitch bonding, and ultrasonic bonding. In some embodiments, the layers are adhered to one another by applying a spray adhesive such as, for example, "3M BRAND SUPER 77 ADHESIVE", available from 3M Company, St. Paul, Minnesota, to one side of the porous abrasive. In other embodiments, a hot-melt adhesive is applied to one side of a layer using either a hot-melt spray gun or an extruder with a comb-type shim. In yet further embodiments, a preformed adhesive mesh is placed between the layers to be joined.

If desired, a seal may be applied to the peripheral edge of the abrasive article, typically to at least a majority (if not all) of the peripheral edge, to reduce or prevent lateral escape of particles not retained by the abrasive article. Examples of seals include welds, tape, latex coatings, caulks, and scalants (e.g., latex or silicone).

Abrasive articles according to the present invention are generally useful for collecting particles during abrading processes, and in some cases, are capable of retaining large amounts of particles at high rates of delivery. The abrasive articles are suitable for use with any devices adapted for use with such articles. Examples include random orbital, dual action, and disc sanders, with or without vacuum applied to the porous attachment layer and/or second nonwoven filter medium of the abrasive article.

Although not wishing to be bound by any particular theory, it is believed that in the case of abrasive articles according to the present invention, the multiple filter components may function such that a given component (e.g., the first nonwoven filter medium) may be aided by a secondary component (e.g., the second nonwoven filter medium) that may address the failure mode of the first component and compensate, keeping overall efficiency high and extending performance to a level that aligns with the performance of the abrasive it is used with.

Accordingly, in some embodiments, at least a portion of an abrasive article (e.g., representative of the perforated area) according to the present invention (in an unused state) exhibits a pressure drop according to the Pressure Drop Measurement Test (hereinbelow) in a range of from 0.2 to 20 millimeters of water. For example, at least a portion of an abrasive article according to the present invention (in an unused state) may exhibits a pressure drop according to the Pressure Drop Measurement Test in a range of from 1 to 15 millimeters of water, or even 4 to 10 millimeters of water.

The Pressure Drop Measurement Test is performed as follows:

Pressure drop across the thickness of an abrasive article is determined using a filter testing apparatus comprising a pair of equal inside diameter cylinders mounted in series, such that, the length of the cylinders is in the vertical direction, and such that air flows through the cylinders with a face velocity of 5.2 centimeters per second. A pressure transducer is mounted to each cylinder to measure the pressure within the cylinders. The adjacent ends of the top and bottom cylinders are sealed upon the abrasive article. The abrasive article being tested is tightly clamped, so as to prevent sideways leakage, between the cylinders with the outer abrasive surface of the abrasive article being perpendicular to the direction of, and facing, the air flow. The difference in air pressure between the first and second cylinders is recorded as the pressure drop of the abrasive article.

Advantages and other embodiments of this invention are further illustrated by the following examples, but the particular materials and amounts thereof recited in these examples, as well as other conditions and details, should not be construed to unduly limit this invention.

Unless otherwise indicated, all parts, percentages, ratios, etc. in the Examples and the rest of the specification are by weight.

### EXAMPLES

The following abbreviations are used throughout the Examples below:

| MATERIALS | |
|---|---|
| IDENTIFICATION | DESCRIPTION |
| AM1 | A non-porous coated abrasive material, commercially available under the trade designation "360L GRADE P800" from 3M Company; St. Paul, Minnesota. |
| AM2 | AM1 laminated to a 13 mil transfer tape, the layered construction laser cut to 5-inch (12.7-cm) diameter discs having a distribution of laser perforated holes prepared according to Procedure 2 (hereinbelow) |
| AM3 | A 6-inch (15.2-cm) diameter porous coated abrasive material, commercially available under the trade designation "NORTON MULTI-AIR, P800" from Norton, Worcester, Massachusetts, die cut to a 5-inch (12.7-cm) diameter disc. |
| AM4 | A grade P320 porous screen abrasive with an integral loop attachment backing, commercially available under the trade designation "ABRANET P320" from KWH Mirka Ltd., Jeppo, Finland. |
| AM5 | An ANSI Grade 500 porous abrasive article, commercially available under the trade designation "3M 281 FABRICUT" from the 3M Company, die cut into 5-inch (12.7-cm) diameter discs. |
| AM6 | A replicate of the screen abrasive described in Example 3 from U.S. Pat. Appl. Publ. No. 2006/0148390 A1 (Woo et al.) |
| FM1 | A nonwoven polyester pad, commercially available under the trade designation "3M CARPET BONNET PAD WHITE" from 3M Company, die cut to a 5-inch (12.7-cm) diameter disc. |
| FM2 | An electret staple fiber web. 150 grams per square meter basis weight, commercially available under the trade designation "FILTRETE G 150" from 3M Company, die cut to a 5-inch (12.7-cm) diameter disc. |
| FM3 | FM1 having the edge sealed with a commercially available caulk, as described in Procedure 1 (hereinbelow). |
| FM4 | A nonwoven filter medium prepared as described in Procedure 6 (hcreinbelow). |
| FM5 | A bimodal blown micro-fiber (BMF) electret polypropylene web, 260 g/m² basis weight, having a thickness of 3.6 mm, prepared generally according to the procedure of Example 1 of U.S. Pat. Appln. No. 11/461136 to Brandner et al., filed July 31, 2006. |
| FM6 | A bimodal blown micro-fiber (BMF) electret polypropylene web, 94 g/m² basis weight, having a thickness of 0.9 mm, prepared generally according to the procedure of Example 1 of U.S. Pat. Appln. No. 11/461136 to Brandner et al., filed July 31, 2006. |
| AT1 | A loop attachment fabric, commercially available under the trade designation "70 G/M² TRICOT DAYTONA BRUSHED NYLON LOOP FABRIC" from Sitip SpA, Gene, Italy. |
| FIB1 | A polyester staple fiber, commercially available under the trade designation "T-240 COPET/PET" from Fiber Innovation Technology Inc. Johnson City, Tennessee. |
| FIB2 | A polyester staple fiber, commercially available under the trade designation "Type 224", 15 Denier, 2.0 inch length available from KoSa, Salisbury, North Carolina. |

### Procedure 1: Filter Medium Edge Scaling

The edge of a disc of filter medium 1, FM1, was sealed by applying a smooth, continuous bead of silicon-acrylic caulking material having the trade designation "DAP ALEX PLUS" manufactured by DAP Products, Inc., Baltimore, Maryland; around the peripheral edge (abutting the circumference) of the disc. The caulk was forced into the edge of the filter medium via a spatula. The caulk was allowed to dry at least 8 hours. FM1, sealed in this manner was designated as FM3.

### Procedure 2: Lamination of Transfer Tape to Abrasive Material and Laser Perforation

A sheet of abrasive material 1, AM 1, was laminated to similar sized sheet of a dual-sided transfer tape having the trade designation "3M 964 13 MIL TRANSFER TAPE" available from the 3M Company, by the following procedure. One side of the tape's liner was removed and the side of a sheet of AM1 opposite the outer abrasive surface was hand-laminated to the exposed, tacky pressure sensitive adhesive of the tape. The laminated abrasive was laser perforated according to pattern 400 shown in Fig. 4. Laser perforated and cut 5-inch diameter discs of this layered construction were designated as AM2.

### Procedure 3: Attachment of Filter Medium or Abrasive Material to AT1

A pressure-sensitive adhesive, commercially available under the trade designation "SUPER 77 SPRAY ADHESIVE" from 3M Company, was applied to the non-loop side of an approximately 6-inch (15.2-cm) square sheet of AT1 and allowed to dry for approximately 30 seconds at 25 degrees Celsius. The dry weight of adhesive was about 12 milligrams per square centimeter (mg/cm²). The circular surface of the filter medium FM1, FM2, or FM3, or abrasive material AM5 or AM6, was laminated to the adhesive coated surface of AT1. The excess material of AT1 protruding from the edge of the construction was removed by cutting with a scissors, creating a circular, substantially coextensive, multi-layer construction.

### Procedure 4: Attachment of Filter Medium to AM2

The liner of the transfer tape of AM2 was removed exposing the tacky, pressure sensitive adhesive of the tape. The appropriate circular disc of filter medium, FM1 or FM3, was aligned with and hand laminated to the adhesive, such that, the layer of AM2 and the layer of filter medium were substantially coextensive.

In some instances, FM1 and FM3 had previously been laminated to a disc of FM2, as reported below. In those cases, the exposed circular surface of FM1 or FM3, i.e., the side opposite the surface attached to FM2, was laminated to AM2.

In the case were AM2 is attached to the FM4/FM5 needle tacked filter medium, AM2 is attached to the exposed circular surface of FM4, forming a substantially coextensive layers.

### Procedure 5: Attachment of FM1 or FM3 to FM2

A pressure-sensitive adhesive, commercially available under the trade designation "SUPER 77 SPRAY ADHESIVE" from 3M Company, was applied to a circular surface of filter medium, FM1 or FM3, and to a circular surface of FM2, and allowed to dry for approximately 30 seconds at 25 degrees Celsius. The dry weight of adhesive was about 12 milligrams per square centimeter (mg/cm²). The two adhesive coated, circular surfaces were then aligned and laminated to one another. The construction was allowed to dry, creating a substantially coextensive, two-layer construction.

### Procedure 6: Fabrication of FM4

FM4 was formed from a 90/10, by weight, blend of FIB 1 and FIB2. The basis weight of the blend was about 155 grains/24 square inch. (648 g/m²), with a thickness of about 5 inches (12 cm). An air laid web former, trade designation "RANDO WEBBER", available from Rando Machine Corporation, Macedon, New York was employed using conventional conditions to form FM4 from the indicated fiber blend..

### Procedure 7: Attachment of FM4 to FM5

Upon exit from the Rando Webber in Procedure 6, FM4 was positioned above FM5 and the two layers were attached to one another by passing them through a needle tacker, trade designation "AUTOMATEX", available from STP Impianti Spa, Milan, Italy, at a speed of 1.52 m/minute. The needle tacker rate was 185 strokes/minute, with a penetration from above of 15 mm, and a punch density of 8.4 punches/cm². Needles were type F20 9-37-9K 15X20x2.5, available from Foster Needle Co., Manitowoc, Wisconsin. The final basis weight for the needle tacked FM5/FM6 filter medium was about 855 g/m² with a thickness of about 5.2 mm. The combined nonwoven structure was passed through a convection oven for a period of 2 minutes at 129 degrees Celsius, where FIB1 bonded the entire structure together. The finished structure was allowed to cool to 25 degrees Celsius.

Using the procedures described above, a variety of multi-layer abrasive filter discs were prepared as designated in Table 1, Table 2, and Table 3. Replicate examples (i.e., replicates of the same construction) are designated by a numeral followed by a letter (e.g., Example 1a, Example 1b, and Example 1c). Replicate comparative examples are designated by a letter followed by a numeral (e.g., Comparative Example A1, Comparative Example A2, and Comparative Example A3). Various properties of some of the medium materials are reported in Table 4.

For any given specific example, the components (e.g., porous abrasive member, filter medium, and porous attachment layer) that are adjacent to one another in the Tables are adjacent to one another in the actual abrasive articles. It will be apparent to one of skill in the art that the processing sequence in which the layers are combined together to form the multi-layer abrasive disc is often not of particular concern, as long as the desired final construction is obtained.

Moreover, it will be realized that when two or more differing filter medium materials are used in the construction of a multi-layer abrasive filter disc, the order in which the filters are placed relative to the abrasive medium may affect the performance of the abrasive article. In this regard, differing filter medium may not be interchangeable within the multilayer construction. This includes the situation where a single filter medium is employed that contains a gradient in its filtering capabilities (e.g., it is substantially non-homogeneous in the direction through which particles to be filtered flow).

### Test Methods

### Sanding Test Method 1

A 5.0-inch (12.7-cm) diameter abrasive disc was weighed and then attached to a 40-hole, 5.0-inch (12.7-cm) diameter by 3/8-inch (0.95-cm) thick foam back up pad, available under the trade designation "3M HOOKIT BACKUP PAD, #20206" from 3M Company. The backup pad and disc assembly was then mounted onto a 5-inch (12.7-cm) diameter, medium finishing, dual-action orbital sander, model 21033. obtained from Dynabrade Corp., Clarence, New York. The abrasive face of the disc was manually brought into contact with a pre-weighed, 18 inches by 30 inches (46 cm by 76 cm) gel-coated fiberglass reinforced plastic panel, obtained from White Bear Boat Works, White Bear Lake, Minnesota. The sander was run at 90 psi (620 kPa) air line pressure and a down force of 10 pounds force (44 N) for 2 cycles of 75 seconds each. An angle of zero degrees to the surface of the workpiece was used. Each cycle consisted of 24 overlapping transverse passes, for a combined 504 inches (12.8 meters) total length, at a tool speed of 6.7 inches per second (17 cm per second) across the panel surface resulting in an evenly sanded area of test panel. After the first sanding cycle, the test panel was cleaned by blowing compressed air across the top of the sanded panel to remove visible dust. The disc was removed from the back up pad and both the panel and disc were weighed. The abrasive was remounted on the back up pad and the 75-second sanding cycle was repeated using the same test panel. The test panel was again cleaned by blowing compressed air across the top of the sanded panel to remove visible dust. The abrasive disc was removed from the back-up pad and both the panel and abrasive disc were weighed. Reported data is after the 2^{nd} sanding cycle, cumulative sanding time of 150 seconds.

The following measurements were made for each sample tested by this method and reported as an average of two test samples per example in Tables 1 and Table 2 as indicated:
"Cut": Weight, in grams, removed from the plastic panel;
"Retain": weight, in grams, of particles collected in the sample disc; and
"DE %": Ratio of the Retain/Cut multiplied by 100.

### Sanding Test Method 2

A 5.0-inch (12.7-cm) abrasive filter disc was weighed, attached to the back up pad and the disc/pad assembly was then mounted to the orbital sander as described in Sanding Test Method 1. The abrasive face of the disc was manually brought into contact with a pre-weighed, 18 inches by 30 inches (45.7 cm by 76.2 cm) gel-coated fiberglass reinforced plastic panel obtained from White Bear Boat Works, White Bear Lake, Minnesota. The sander was run at 90 psi (620 kPa) air line pressure for 6 cycles of 25 seconds each. An angle of zero degrees to the surface of the workpiece was used. After the first 3 cycles, the test panel was cleaned by blowing compressed air across the top of the sanded panel to remove visible dust. The disc was removed from the back up pad and both the panel and disc were weighed. The abrasive was remounted on the back up pad and the final 3 sanding cycles were conducted using the same test panel. The test panel was again cleaned by blowing compressed air across the top of the sanded panel to remove visible dust. The abrasive disc was removed from the back up pad and both the panel and abrasive disc were weighed. Reported data is after the 6^{th} sanding cycle, cumulative sanding time of 150 seconds.

The following measurements were made for each sample tested by this method and reported as an average of two test samples per example in Tables 1 and Table 2 as indicated:
"Cut": Weight, in grams, removed from the plastic panel;
"Retain": weight, in grams, of particles collected in the sample disc; and
"DE %": Ratio of the Retain/Cut multiplied by 100.

### Surface Finish Measurement Test Method

The resulting surface roughness of the abraded test panels was determined by using a surface finish testing device available under the trade designation "PERTHOMETER MODEL M4P-130589" from Mahr Corporation, Cincinnati, Ohio. Surface finish values were measured at three abraded sections of the test panel after each completed 150-second sanding test. The Rz (also known as Rtm), which is the mean of the maximum peak-to-valley values, was recorded for each measurement.

### Modified Pressure Drop Measurement Test

The Pressure Drop Measurement Test given herein above was carried out using a filter testing apparatus comprising a pair of 4.5-inch (11.4-cm) inside diameter cylinders with an air flow rate of 32 liters per minute. Pressure transducers were obtained from MKS Instruments, Wilmington, Massachusetts under the trade designation "MKS BARATRON PRESSURE TRANSDUCER, 398HD-00010SP12" (10 torr (1.33 kPa) range).

Sanding Test 1 was used as the abrading procedure corresponding to the data generated in Table 1. Sanding Test 2 was used as the abrading procedure corresponding to the data generated in Table 2.

Modified Pressure Drop Test measurements were not made on all examples. Modified Pressure Drop Test for certain Examples reported in Tables 1 and 2 are reported in Table 3 along with data associated with additional comparative examples.

Modified Pressure Drop Test measurement were taken on abrasive articles prior to any abrading conducted via Sanding Test Method 1 or Sanding Test Method 2, with exceptions noted in Table 3.

**TABLE 1**

| | ABRASIVE MEMBER | FIRST FILTER MEDIUM | SECOND FILTER MEDIUM | POROUS ATTACHMENT LAYER | Cut, grams | Retain, grams | DE, percent | Rz, micrometers |
|---|---|---|---|---|---|---|---|---|
| Example 1a | AM2 | FM1 | FM2 | none | 2.44 | 1.81 | 74 | 1.2 |
| Example 2a | AM2 | FM3 | FM2 | none | 2.30 | 1.49 | 65 | 1.4 |
| Example 3a | AM2 | FM1 | FM2 | AT1 | 2.41 | 1.89 | 78 | 1.3 |
| Example 4a | AM2 | FM3 | FM2 | AT1 | 2.49 | 1.86 | 75 | 1.4 |
| Example 5 | AM2 | FM4 | FM5 | none | 2.42 | 2.34 | 97 | 1.4 |
| Comparative Example A1 | AM3 | none | none | none | 4.38 | 0.09 | 2 | 1.9 |
| Comparative Example A4 | AM3 | none | none | none | 3.70 | 0.79 | 21 | 1.9 |

**TABLE 2**

| | ABRASIVE MEMBER | FIRST FILTER MEDIUM | SECOND FILTER MEDIUM | POROUS ATTACHMENT LAYER | Cut, grams | Retain, grams | DE, percent | Rz, micrometers |
|---|---|---|---|---|---|---|---|---|
| Example 1b | AM2 | FM1 | FM2 | none | 2.95 | 2.71 | 92 | 1.5 |
| Example 2b | AM2 | FM3 | FM2 | none | 3.24 | 2.97 | 92 | 1.3 |
| Example 3b | AM2 | FM1 | FM2 | AT1 | 3.04 | 2.83 | 93 | 1.5 |
| Example 4b | AM2 | FM3 | FM2 | AT1 | 2.79 | 2.58 | 92 | 1.5 |
| Example 6 | AM2 | FM1 | FM6 | AT1 | 5.64 | 4.38 | 78 | 1.6 |
| Example 7 | AM2 | FM3 | FM6 | AT1 | 4.51 | 3.86 | 86 | 1.7 |
| Comparative Example A2 | AM3 | none | none | none | 3.57 | 0.07 | 2 | 2.1 |
| Comparative Example A3 | AM3 | none | none | none | 6.80 | 0.07 | 1 | 2.2 |

Examples 1b, 2b, 3b, 4b and Comparative Example A2 were all run using the same gel-coated fiberglass reinforced plastic panel. Examples 6, 7 and Comparative Example A3 were all run using the same gel-coated fiberglass reinforced plastic panel, yet a different panel from the previous examples and comparative example. Example 5 and Comparative Example A4 were run on yet another panel. Variability in the panel can lead to variability in the measured cut.

**TABLE 3**

| | ABRASIVE MEMBER | FIRST FILTER MEDIUM | SECOND FILTER MEDIUM | POROUS ATTACHMENT LAYER | ΔP (MM H₂O) |
|---|---|---|---|---|---|
| Example 1c | AM2 | FM1 | FM2 | none | 1.25 |
| Example 3c | AM2 | FM3 | FM2 | ΔT1 | 1.72 |
| Example 1b* | AM2 | FM1 | FM2 | none | 5.00 |
| Example 3b* | AM2 | FM1 | FM2 | AT1 | 9.13 |
| Example 5 | AM2 | FM4 | FM5 | none | 2.04 |
| Example 6 | AM2 | FM1 | FM6 | AT1 | 2.09 |
| Example 7 | AM2 | FM3 | FM6 | AT1 | 2.33 |
| Comparative Example A3 | AM3 | none | none | none | 0.06 |
| Comparative Example B | AM4 | none | none | none | 0.03 |
| Comparative Example C | AM5 | none | none | none | 0.03 |
| Comparative Example D | AM5 | none | none | AT1 | 0.09 |
| Comparative Example E | AM6 | none | none | none | 0.03 |
| Comparative Example F | AM6 | none | none | AT1 | 0.10 |
| Comparative Example G | AM2 | FM1 | none | none | 0.38 |
| Comparative Example H | AM2 | FM1 | none | AT1 | 0.71 |

| | | | | | |
|---|---|---|---|---|---|
| * Examples 1b and 3b in Table 3 (above) were measured after Sanding Test Method 2 was completed. | | | | | |

**TABLE4**

| MEDIUM | BASIS WEIGHT, grams per square meter | CALIPER, centimeters | BULK DENSITY, g/cm³ | FIBER DIAMETER, micrometers |
|---|---|---|---|---|
| FM1 | 482 (461-503) | 0.706 (0.67-0.74) | 0.068 | 30 |
| FM2 | 150 | 0.25 | 0.060 | 12x12 to 12x25 |
| FM5 | 260 | 0.36 | 0.072 | 29 average (bimodal) |
| FM6 | 94 | 0.087 | 0.107 | 22 average (bimodal) |
| AT1 | 70 | 0.045 | 0.156 | not determined |

Various modifications and alterations of this invention may be made by those skilled in the art without departing from the scope of this invention, and it should be understood that this invention is not to be unduly limited to the illustrative embodiments set forth herein.

## Claims

1. An abrasive article comprising:
a porous abrasive member comprising: an abrasive layer proximate and affixed to a first surface of a substrate, the abrasive layer comprising a plurality of abrasive particles affixed to the first surface of the substrate by at least one binder, wherein the abrasive layer has an outer abrasive surface, wherein the substrate has a second surface opposite the first surface of the substrate, and wherein a plurality of openings extend from the outer abrasive surface to the second surface of the substrate;
a first nonwoven filter medium having a first surface and a second surface opposite the first surface, wherein the first surface of the first nonwoven filter medium is proximate and affixed to the second surface of the substrate, wherein the first nonwoven filter medium comprises a plurality of fibers; and
a second nonwoven filter medium having a first surface and a second surface opposite the first surface, wherein the first surface of the second nonwoven filter medium is proximate and affixed to the second surface of the first nonwoven filter medium, and wherein the second nonwoven filter medium comprises a plurality of fibers;
wherein the plurality of openings cooperate with the first nonwoven filter medium to allow the flow of particles from the outer abrasive surface to the second nonwoven filter medium, and wherein, in an unused state, the at least a portion of the abrasive article exhibits a pressure drop according to the Pressure Drop Measurement Test in a range of from 0.2 to 20 millimeters of water.

2. An abrasive article according to claim 1, wherein the porous abrasive member comprises an apertured coated abrasive.

3. An abrasive article according to claim 1, further comprising a porous attachment layer proximate and affixed to the second surface of the second nonwoven filter medium.

4. An abrasive article according to claim 1, wherein at least one of the first or second nonwoven filter medium has a peripheral edge that is scaled along a major portion thereof.

5. A method of abrading a surface of a workpiece, the method comprising contacting the surface with an abrasive article according to claim 1, and relatively moving the abrasive article and the surface to mechanically modify the surface.

6. A method of making an abrasive article, the method comprising:
providing a porous abrasive member comprising: an abrasive layer proximate and affixed to a first surface of a substrate, the abrasive layer comprising a plurality of abrasive particles affixed to the first surface of the substrate by at least one binder, wherein the abrasive layer has an outer abrasive surface, wherein the substrate has a second surface opposite the first surface of the substrate, and wherein a plurality of openings extend from the outer abrasive surface to the second surface of the substrate;
providing a first nonwoven filter medium, the first nonwoven filter medium having a first surface and a second surface opposite the first surface, wherein the first nonwoven filter medium comprises a plurality of fibers, and wherein the first surface of the first nonwoven filter medium is proximate the second surface of the substrate;
providing a second nonwoven filter medium, the second nonwoven filter medium having a first surface and a second surface opposite the first surface, wherein the second nonwoven filter medium comprises a plurality of fibers, and wherein the first surface of the second nonwoven filter medium is proximate the second surface of the first nonwoven filter medium;
affixing the first nonwoven filter medium to the second surface of the substrate;
and
affixing the second nonwoven filter medium to the first nonwoven filter medium;
wherein the plurality of openings cooperate with the first nonwoven filter medium to allow the flow of particles from the outer abrasive surface to the second nonwoven filter medium, and wherein, in an unused state, at least a portion of the abrasive article exhibits a pressure drop according to the Pressure Drop Measurement Test in a range of from 0.2 to 20 millimeters of water.

7. A method of making an abrasive article according to claim 6, wherein the porous abrasive member comprises an apertured coated abrasive.

8. A method of making an abrasive article according to claim 6, the method further comprising sealing a major portion of a peripheral edge of at least one of the first or second nonwoven filter medium.

9. A method of making an abrasive article according to claim 6, further comprising affixing a porous attachment layer to the second nonwoven filter medium.

10. An abrasive article comprising:
a porous abrasive member comprising: an abrasive layer proximate and affixed to a first surface of a substrate, the abrasive layer comprising a plurality of abrasive particles affixed to the first surface of the substrate by at least one binder, wherein the abrasive layer has an outer abrasive surface, wherein the substrate has a second surface opposite the first surface of the substrate, and wherein a plurality of openings extend from the outer abrasive surface to the second surface of the substrate;
a first nonwoven filter medium having a first surface and a second surface opposite the first surface, wherein the first surface of the first nonwoven filter medium is proximate and affixed to the second surface of the substrate, wherein the first nonwoven filter medium comprises a plurality of fibers, and wherein the first nonwoven filter medium has a thickness of from 1 to 25 millimeters and a density of from 0.04 to 0.5 grams per cubic centimeter; and
a second nonwoven filter medium having a first surface and a second surface opposite the first surface, wherein the first surface of the second nonwoven filter medium is proximate and affixed to the second surface of the first nonwoven filter medium, wherein the second nonwoven filter medium comprises a plurality of fibers, and wherein the second nonwoven filter medium has a thickness of from 0.5 to 15 millimeters and a bulk density of from 0.04 to 0.5 grams per cubic centimeter; and
wherein the plurality of openings cooperate with the first nonwoven filter medium to allow the flow of particles from the outer abrasive surface to the second nonwoven filter medium.

11. An abrasive article according to claim 10, wherein the porous abrasive member comprises an apertured coated abrasive.

12. An abrasive article according to claim 10, further comprising a porous attachment layer proximate and affixed to the second surface of the second nonwoven filter medium.

13. An abrasive article according to claim 10, wherein at least one of the first or second nonwoven filter medium has a peripheral edge that is sealed along a major portion thereof.

14. A method of abrading a surface of a workpiece, the method comprising contacting the surface with an abrasive article according to claim 10, and relatively moving the abrasive article and the surface to mechanically modify the surface.

15. A method of making an abrasive article, the method comprising:
providing a porous abrasive member comprising: an abrasive layer proximate and affixed to a first surface of a substrate, the abrasive layer comprising a plurality of abrasive particles affixed to the first surface of the substrate by at least one binder, wherein the abrasive layer has an outer abrasive surface, wherein the substrate has a second surface opposite the first surface of the substrate, and wherein a plurality of openings extend from the outer abrasive surface to the second surface of the substrate;
providing a first nonwoven filter medium having a first surface and a second surface opposite the first surface, wherein the first surface of the first nonwoven filter medium is proximate the second surface of the substrate, wherein the first nonwoven filter medium comprises a plurality of fibers, and wherein the second nonwoven filter medium has a thickness of from 0.5 to 15 millimeters and a bulk density of from 0.04 to 0.5 grams per cubic centimeter;
providing a second nonwoven filter medium having a first surface and a second surface opposite the first surface, wherein the first surface of the second nonwoven filter medium is proximate the second surface of the first nonwoven filter medium, wherein the second nonwoven filter medium comprises a plurality of fibers, wherein the second nonwoven filter medium has a thickness of from 0.5 to 15 millimeters and a bulk density of from 0.04 to 0.5 grams per cubic centimeter;
affixing the first nonwoven filter medium to the second surface of the substrate,
and
affixing the second nonwoven filter medium to the first nonwoven filter medium,
wherein the plurality of openings cooperate with the first nonwoven filter medium to allow the flow of particles from the outer abrasive surface to the second nonwoven filter medium.

16. A method of making an abrasive article according to claim 15, wherein the porous abrasive member comprises an apertured coated abrasive.

17. A method of making an abrasive article according to claim 15, the method further comprising sealing a major portion of a peripheral edge of at least one of the first or second nonwoven filter medium.

18. A method of making an abrasive article according to claim 15, further comprising affixing a porous attachment layer to the second nonwoven filter medium.

## Patentansprüche

1. Schleifgegenstand, Folgendes umfassend:
ein poröses Schleifelement, Folgendes umfassend: eine Schleifschicht, unmittelbar an einer ersten Oberfläche eines Substrats liegend und daran befestigt, wobei die Schleifschicht mehrere Schleifpartikel umfasst, die durch mindestens ein Bindemittel an der ersten Oberfläche des Substrats befestigt sind, wobei die Schleifschicht eine äußere Schleifoberfläche aufweist, wobei das Substrat eine zweite Oberfläche gegenüber der ersten Oberfläche des Substrats aufweist und wobei sich mehrere Öffnungen von der äußeren Schleifoberfläche zur zweiten Oberfläche des Substrats erstrecken,
ein erstes Vliesfiltermedium, das eine erste Oberfläche und eine zweite Oberfläche gegenüber der ersten Oberfläche aufweist, wobei die erste Oberfläche des ersten Vliesfiltermediums unmittelbar an der zweiten Oberfläche des Substrats liegt und daran befestigt ist, wobei das erste Vliesfiltermedium mehrere Fasern umfasst, und
ein zweites Vliesfiltermedium, das eine erste Oberfläche und eine zweite Oberfläche gegenüber der ersten Oberfläche aufweist, wobei die erste Oberfläche des zweiten Vliesfiltermediums unmittelbar an der zweiten Oberfläche des ersten Vliesfiltermediums liegt und daran befestigt ist und wobei das zweite Vliesfiltermedium mehrere Fasern umfasst, und
wobei die mehreren Öffnungen mit dem ersten Vliesfiltermedium zusammenwirken, um das Strömen von Partikeln von der äußeren Schleifoberfläche zum zweiten Vliesfiltermedium zu ermöglichen und wobei in einem Zustand des Nichtgebrauchs der mindestens eine Abschnitt des Schleifgegenstandes gemäß der Druckverlustprüfung einen Druckverlust im Bereich von 0,2 bis 20 Millimetern Wasser aufweist.

2. Schleifgegenstand nach Anspruch 1, wobei das poröse Schleifelement ein mit Öffnungen versehenes, beschichtetes Schleifmittel umfasst.

3. Schleifgegenstand nach Anspruch 1, weiterhin umfassend eine poröse Befestigungsschicht, unmittelbar an der zweiten Oberfläche des zweiten Vliesfiltermediums liegend und daran befestigt.

4. Schleifgegenstand nach Anspruch 1, wobei mindestens eins des ersten oder Vliesfiltermediums einen Außenrand aufweist, der über einen größeren Teil davon versiegelt ist.

5. Verfahren zum Schleifen einer Oberfläche eines Werkstücks, wobei das Verfahren das In-Kontakt-Bringen der Oberfläche mit einem Schleifgegenstand nach Anspruch 1 und das Bewegen des Schleifgegenstandes und der Oberfläche im Verhältnis zueinander umfasst, um die Oberfläche mechanisch zu modifizieren.

6. Verfahren zur Herstellung eines Schleifgegenstandes, wobei das Verfahren Folgendes umfasst:
Bereitstellen eines porösen Schleifelements, Folgendes umfassend: eine Schleifschicht, unmittelbar an einer ersten Oberfläche eines Substrats liegend und daran befestigt, wobei die Schleifschicht mehrere Schleifpartikel umfasst, die durch mindestens ein Bindemittel an der ersten Oberfläche des Substrats befestigt sind, wobei die Schleifschicht eine äußere Schleifoberfläche aufweist, wobei das Substrat eine zweite Oberfläche gegenüber der ersten Oberfläche des Substrats aufweist und wobei sich mehrere Öffnungen von der äußeren Schleifoberfläche zur zweiten Oberfläche des Substrats erstrecken,
Bereitstellen eines ersten Vliesfiltermediums, wobei das erste Vliesfiltermedium eine erste Oberfläche und eine zweite Oberfläche gegenüber der ersten Oberfläche aufweist, wobei das erste Vliesfiltermedium mehrere Fasern umfasst, und wobei die erste Oberfläche des ersten Vliesfiltermediums unmittelbar an der zweiten Oberfläche des Substrats liegt,
Bereitstellen eines zweiten Vliesfiltermediums, wobei das zweite Vliesfiltermedium eine erste Oberfläche und eine zweite Oberfläche gegenüber der ersten Oberfläche aufweist, wobei das zweite Vliesfiltermedium mehrere Fasern umfasst, und wobei die erste Oberfläche des zweiten Vliesfiltermediums unmittelbar an der zweiten Oberfläche des ersten Vliesfiltermediums liegt,
Befestigen des ersten Vliesfiltermediums an der zweiten Oberfläche des Substrats und
Befestigen des zweiten Vliesfiltermediums an dem ersten Vliesfiltermedium,
wobei die mehreren Öffnungen mit dem ersten Vliesfiltermedium zusammenwirken, um das Strömen von Partikeln von der äußeren Schleifoberfläche zum zweiten Vliesfiltermedium zu ermöglichen und wobei in einem Zustand des Nichtgebrauchs mindestens ein Abschnitt des Schleifgegenstandes gemäß der Druckverlustprüfung einen Druckverlust im Bereich von 0,2 bis 20 Millimetern Wasser aufweist.

7. Verfahren zur Herstellung eines Schleifgegenstandes nach Anspruch 6, wobei das poröse Schleifelement ein mit Öffnungen versehenes, beschichtetes Schleifmittel umfasst.

8. Verfahren zur Herstellung eines Schleifgegenstandes nach Anspruch 6, wobei das Verfahren ferner das Versiegeln eines größeren Teils eines Außenrandes des ersten oder zweiten Vliesfiltermediums umfasst.

9. Verfahren zur Herstellung eines Schleifgegenstandes nach Anspruch 6, weiterhin umfassend das Befestigen einer porösen Befestigungsschicht an dem zweiten Vliesfiltermedium.

10. Schleifgegenstand, Folgendes umfassend:
ein poröses Schleifelement, Folgendes umfassend: eine Schleifschicht, unmittelbar an einer ersten Oberfläche eines Substrats liegend und daran befestigt, wobei die Schleifschicht mehrere Schleifpartikel umfasst, die durch mindestens ein Bindemittel an der ersten Oberfläche des Substrats befestigt sind, wobei die Schleifschicht eine äußere Schleifoberfläche aufweist, wobei das Substrat eine zweite Oberfläche gegenüber der ersten Oberfläche des Substrats aufweist und wobei sich mehrere Öffnungen von der äußeren Schleifoberfläche zur zweiten Oberfläche des Substrats erstrecken,
ein erstes Vliesfiltermedium, das eine erste Oberfläche und eine zweite Oberfläche gegenüber der ersten Oberfläche aufweist, wobei die erste Oberfläche des ersten Vliesfiltermediums unmittelbar an der zweiten Oberfläche des Substrats liegt und daran befestigt ist, wobei das erste Vliesfiltermedium mehrere Fasern umfasst und wobei das erste Vliesfiltermedium eine Dicke von 1 bis 25 Millimetern und eine Dichte von 0,04 bis 0,5 Gramm pro Kubikzentimeter aufweist, und
ein zweites Vliesfiltermedium, das eine erste Oberfläche und eine zweite Oberfläche gegenüber der ersten Oberfläche aufweist, wobei die erste Oberfläche des zweiten Vliesfiltermediums unmittelbar an der zweiten Oberfläche des ersten Vliesfiltermediums liegt und daran befestigt ist, wobei das Vliesfiltermedium mehrere Fasern umfasst, und wobei das zweite Vliesfiltermedium eine Dicke von 0,5 bis 15 Millimetern und eine Fülldichte von 0,04 bis 0,5 Gramm pro Kubikzentimeter aufweist, und
wobei die mehreren Öffnungen mit dem ersten Vliesfiltermedium zusammenwirken, um das Strömen von Partikeln von der äußeren Schleifoberfläche zum zweiten Vliesfiltermedium zu ermöglichen.

11. Schleifgegenstand nach Anspruch 10, wobei das poröse Schleifelement ein mit Öffnungen versehenes, beschichtetes Schleifmittel umfasst.

12. Schleifgegenstand nach Anspruch 10, weiterhin umfassend eine poröse Befestigungsschicht, unmittelbar an der zweiten Oberfläche des zweiten Vliesfiltermediums liegend und daran befestigt.

13. Schleifgegenstand nach Anspruch 10, wobei mindestens eins des ersten oder zweiten Vliesfiltermediums einen Außenrand aufweist, der über einen größeren Teil davon versiegelt ist.

14. Verfahren zum Schleifen einer Oberfläche eines Werkstücks, wobei das Verfahren das In-Kontakt-Bringen der Oberfläche mit einem Schleifgegenstand nach Anspruch 10 und das Bewegen des Schleifgegenstandes und der Oberfläche in Verhältnis zueinander umfasst, um die Oberfläche mechanisch zu modifizierten.

15. Verfahren zur Herstellung eines Schleifgegenstandes, wobei das Verfahren Folgendes umfasst:
Bereitstellen eines porösen Schleifelements, Folgendes umfassend: eine Schleifschicht, unmittelbar an einer ersten Oberfläche eines Substrats liegend und daran befestigt, wobei die Schleifschicht mehrere Schleifpartikel umfasst, die durch mindestens ein Bindemittel an der ersten Oberfläche des Substrats befestigt sind, wobei die Schleifschicht eine äußere Schleifoberfläche aufweist, wobei das Substrat eine zweite Oberfläche gegenüber der ersten Oberfläche des Substrats aufweist und wobei sich mehrere Öffnungen von der äußeren Schleifoberfläche zur zweiten Oberfläche des Substrats erstrecken,
Bereitstellen eines ersten Vliesfiltermediums, das eine erste Oberfläche und eine zweite Oberfläche gegenüber der ersten Oberfläche aufweist, wobei die erste Oberfläche des ersten Vliesfiltermediums unmittelbar an der zweiten Oberfläche des Substrats liegt, wobei das erste Vliesfiltermedium mehrere Fasern aufweist, wobei das zweite Vliesfiltermedium eine Dicke von 0,5 bis 15 Millimetern und eine Fülldichte von 0,04 bis 0,5 Gramm pro Kubikzentimeter aufweist,
Bereitstellen eines zweiten Vliesfiltermediums, das eine erste Oberfläche und eine zweite Oberfläche gegenüber der ersten Oberfläche aufweist, wobei die erste Oberfläche des zweiten Vliesfiltermediums unmittelbar an der zweiten Oberfläche des ersten Vliesfiltermediums liegt, wobei das Vliesfiltermedium mehrere Fasern umfasst, wobei das zweite Vliesfiltermedium eine Dicke von 0,5 bis 15 Millimetern und eine Fülldichte von 0,04 bis 0,5 Gramm pro Kubikzentimeter aufweist,
Befestigen des ersten Vliesfiltermediums an der zweiten Oberfläche des Substrats und
Befestigen des zweiten Vliesfiltermediums an dem ersten Vliesfiltermedium,
wobei die mehreren Öffnungen mit dem ersten Vliesfiltermedium zusammenwirken, um das Strömen von Partikeln von der äußeren Schleifoberfläche zum zweiten Vliesfiltermedium zu ermöglichen.

16. Verfahren zur Herstellung eines Schleifgegenstandes nach Anspruch 15, wobei das poröse Schleifelement ein mit Öffnungen versehenes, beschichtetes Schleifmittel umfasst.

17. Verfahren zur Herstellung eines Schleifgegenstandes nach Anspruch 15, wobei das Verfahren ferner das Versiegeln eines größeren Teils eines Außenrandes mindestens eines des ersten oder zweiten Vliesfiltermediums umfasst.

18. Verfahren zur Herstellung eines Schleifgegenstandes nach Anspruch 15, weiterhin umfassend das Befestigen einer porösen Befestigungsschicht an dem zweiten Vliesfiltermedium.

## Revendications

1. Article abrasif comprenant :
un élément abrasif poreux comprenant : une couche abrasive proximale et fixée à une première surface d'un substrat, la couche abrasive comprenant une pluralité de particules abrasives fixées à la première surface du substrat par au moins un liant, dans lequel la couche abrasive comporte une surface abrasive extérieure, dans lequel le substrat comporte une deuxième surface opposée à la première surface du substrat, et dans lequel une pluralité d'ouvertures s'étendent de la surface abrasive extérieure à la deuxième surface du substrat ;
un premier matériau filtrant non tissé comportant une première surface et une deuxième surface opposée à la première surface, la première surface du premier matériau filtrant non tissé étant proximale et fixée à la deuxième surface du substrat et le premier matériau filtrant non tissé comprenant une pluralité de fibres ; et
un deuxième matériau filtrant non tissé comportant une première surface et une deuxième surface opposée à la première surface, la première surface du deuxième matériau filtrant non tissé étant proximale et fixée à la deuxième surface du premier matériau filtrant non tissé, et le deuxième matériau filtrant non tissé comprenant une pluralité de fibres ;
dans lequel la pluralité d'ouvertures coopèrent avec le premier matériau filtrant non tissé pour permettre l'écoulement de particules de la surface abrasive extérieure au deuxième matériau filtrant non tissé, et dans lequel, dans un état inutilisé, l'au moins une portion de l'article abrasif présente une chute de pression, selon l'Essai de mesure de chute de pression, de 0,2 à 20 millimètres d'eau.

2. Article abrasif selon la revendication 1, dans lequel l'élément abrasif poreux comprend un abrasif revêtu pourvu d'ouvertures.

3. Article abrasif selon la revendication 1, comprenant en outre une couche de fixation poreuse proximale et fixée à la deuxième surface du deuxième matériau filtrant non tissé.

4. Article abrasif selon la revendication 1, dans lequel au moins un du premier matériau filtrant non tissé ou du deuxième matériau filtrant non tissé comporte un bord périphérique qui est étanché le long d'une portion majeure de celui-ci.

5. Procédé d'abrasion d'une surface d'une pièce à usiner, le procédé comprenant la mise en contact de la surface avec un article abrasif selon la revendication 1, et le déplacement de l'article abrasif et de la surface l'un par rapport à l'autre pour modifier mécaniquement la surface.

6. Procédé de fabrication d'un article abrasif, le procédé comprenant :
la fourniture d'un élément abrasif poreux comprenant : une couche abrasive proximale et fixée à une première surface d'un substrat, la couche abrasive comprenant une pluralité de particules abrasives fixées à la première surface du substrat par au moins un liant, dans lequel la couche abrasive comporte une surface abrasive extérieure, dans lequel le substrat comporte une deuxième surface opposée à la première surface du substrat, et dans lequel une pluralité d'ouvertures s'étendent de la surface abrasive extérieure à la deuxième surface du substrat ;
la fourniture d'un premier matériau filtrant non tissé, le premier matériau filtrant non tissé comportant une première surface et une deuxième surface opposée à la première surface, le premier matériau filtrant non tissé comprenant une pluralité de fibres, et la première surface du premier matériau filtrant non tissé étant proximale à la deuxième surface du substrat ;
la fourniture d'un deuxième matériau filtrant non tissé, le deuxième matériau filtrant non tissé comportant une première surface et une deuxième surface opposée à la première surface, le deuxième matériau filtrant non tissé comprenant une pluralité de fibres, et la première surface du deuxième matériau filtrant non tissé étant proximale à la deuxième surface du premier matériau filtrant non tissé ;
la fixation du premier matériau filtrant non tissé à la deuxième surface du substrat ; et
la fixation du deuxième matériau filtrant non tissé au premier matériau filtrant non tissé ;
dans lequel la pluralité d'ouvertures coopèrent avec le premier matériau filtrant non tissé pour permettre l'écoulement de particules de la surface abrasive extérieure au deuxième matériau filtrant non tissé, et dans lequel, dans un état inutilisé, au moins une portion de l'article abrasif présente une chute de pression, selon l'Essai de mesure de chute de pression, de 0,2 à 20 millimètres d'eau.

7. Procédé de fabrication d'un article abrasif selon la revendication 6, dans lequel l'élément abrasif poreux comprend un abrasif revêtu pourvu d'ouvertures.

8. Procédé de fabrication d'un article abrasif selon la revendication 6, le procédé comprenant en outre l'étanchement d'une portion majeure d'un bord périphérique d'au moins un du premier matériau filtrant non tissé ou du deuxième matériau filtrant non tissé.

9. Procédé de fabrication d'un article abrasif selon la revendication 6, comprenant en outre la fixation d'une couche de fixation poreuse au deuxième matériau filtrant non tissé.

10. Article abrasif comprenant :
un élément abrasif poreux comprenant : une couche abrasive proximale et fixée à une première surface d'un substrat, la couche abrasive comprenant une pluralité de particules abrasives fixées à la première surface du substrat par au moins un liant, dans lequel la couche abrasive comporte une surface abrasive extérieure, dans lequel le substrat comporte une deuxième surface opposée à la première surface du substrat, et dans lequel une pluralité d'ouvertures s'étendent de la surface abrasive extérieure à la deuxième surface du substrat ;
un premier matériau filtrant non tissé comportant une première surface et une deuxième surface opposée à la première surface, la première surface du premier matériau filtrant non tissé étant proximale et fixée à la deuxième surface du substrat, le premier matériau filtrant non tissé comprenant une pluralité de fibres, et dans lequel le premier matériau filtrant non tissé a une épaisseur de 1 à 25 millimètres et une densité de 0,04 à 0,5 gramme par centimètre cube ; et
un deuxième matériau filtrant non tissé comportant une première surface et une deuxième surface opposée à la première surface, la première surface du deuxième matériau filtrant non tissé étant proximale et fixée à la deuxième surface du premier matériau filtrant non tissé, le deuxième matériau filtrant non tissé comprenant une pluralité de fibres, et dans lequel le deuxième matériau filtrant non tissé a une épaisseur de 0,5 à 15 millimètres et une densité apparente de 0,04 à 0,5 gramme par centimètre cube ; et
dans lequel la pluralité d'ouvertures coopèrent avec le premier matériau filtrant non tissé pour permettre l'écoulement de particules de la surface abrasive extérieure au deuxième matériau filtrant non tissé.

11. Article abrasif selon la revendication 10, dans lequel l'élément abrasif poreux comprend un abrasif revêtu pourvu d'ouvertures.

12. Article abrasif selon la revendication 10, comprenant en outre une couche de fixation poreuse proximale et fixée à la deuxième surface du deuxième matériau filtrant non tissé.

13. Article abrasif selon la revendication 10, dans lequel au moins un du premier matériau filtrant non tissé ou du deuxième matériau filtrant non tissé comporte un bord périphérique qui est étanché le long d'une portion majeure de celui-ci.

14. Procédé d'abrasion d'une surface d'une pièce à usiner, le procédé comprenant la mise en contact de la surface avec un article abrasif selon la revendication 10, et le déplacement de l'article abrasif et de la surface l'un par rapport à l'autre pour modifier mécaniquement la surface.

15. Procédé de fabrication d'un article abrasif, le procédé comprenant :
la fourniture d'un élément abrasif poreux comprenant : une couche abrasive proximale et fixée à une première surface d'un substrat, la couche abrasive comprenant une pluralité de particules abrasives fixées à la première surface du substrat par au moins un liant, dans lequel la couche abrasive comporte une surface abrasive extérieure, dans lequel le substrat comporte une deuxième surface opposée à la première surface du substrat, et dans lequel une pluralité d'ouvertures s'étendent de la surface abrasive extérieure à la deuxième surface du substrat ;
la fourniture d'un premier matériau filtrant non tissé comportant une première surface et une deuxième surface opposée à la première surface, la première surface du premier matériau filtrant non tissé étant proximale à la deuxième surface du substrat, le premier matériau filtrant non tissé comprenant une pluralité de fibres, et dans lequel le deuxième matériau filtrant non tissé a une épaisseur de 0,5 à 15 millimètres et une densité apparente de 0,04 à 0,5 gramme par centimètre cube ;
la fourniture d'un deuxième matériau filtrant non tissé comportant une première surface et une deuxième surface opposée à la première surface, la première surface du deuxième matériau filtrant non tissé étant proximale à la deuxième surface du premier matériau filtrant non tissé, le deuxième matériau filtrant non tissé comprenant une pluralité de fibres, et dans lequel le deuxième matériau filtrant non tissé a une épaisseur de 0,5 à 15 millimètres et une densité apparente de 0,04 à 0,5 gramme par centimètre cube ;
la fixation du premier matériau filtrant non tissé à la deuxième surface du substrat ; et
la fixation du deuxième matériau filtrant non tissé au premier matériau filtrant non tissé ;
dans lequel la pluralité d'ouvertures coopèrent avec le premier matériau filtrant non tissé pour permettre l'écoulement de particules de la surface abrasive extérieure au deuxième matériau filtrant non tissé.

16. Procédé de fabrication d'un article abrasif selon la revendication 15, dans lequel l'élément abrasif poreux comprend un abrasif revêtu pourvu d'ouvertures.

17. Procédé de fabrication d'un article abrasif selon la revendication 15, le procédé comprenant en outre l'étanchement d'une portion majeure d'un bord périphérique d'au moins un du premier matériau filtrant non tissé ou du deuxième matériau filtrant non tissé.

18. Procédé de fabrication d'un article abrasif selon la revendication 15, comprenant en outre la fixation d'une couche de fixation poreuse au deuxième matériau filtrant non tissé.
